# EUROPEAN PATENT SPECIFICATION

(11) **EP 0 869 855 B1**
(45) Date of publication and mention of the grant of the patent: **23.03.2005**
(21) Application number: 95939851.2
(22) Date of filing: 27.11.1995
(51) Int. Cl.: B22D 19/14

(54) **MMC AND LIQUID METAL INFILTRATION PROCESS**
MMC UND FLÜSSIGMETALLINFILTRATIONSVERFHREN
CMM ET PROCEDE D'INTRODUCTION D'UN METAL LIQUIDE PAR INFILTRATION

(43) Date of publication of application: 14.10.1998
(73) Proprietor: Chesapeake Composites Corporation, New Castle, DE 19720 (US)
(72) Inventor: BROWN, Alexander, M., Wilmington, DE 19808 (US); KLIER, Eric, M., Catonsville, MD 21228 (US)
(74) Representative: Turi, Michael, Dipl.-Phys.
(86) International application number: PCT/US1995/014557
(87) International publication number: WO 1997/019774

(56) References cited:
- US-A- 4 710 348
- US-A- 4 915 908
- US-A- 4 985 202
- US-A- 5 111 871
- US-A- 5 196 273
- COMPOSITES, Vol. 23, No. 1, January 1992, SHANKER et al., "Properties of TaC-BASED Metal-Matrix Composites Produced by Melt Infiltration", pages 47-53.

## Description

### FIELD OF THE INVENTION

This invention relates to the manufacture of metalceramic composites having a high tensile modulus, good ductility, toughness, formability, and machinability, and more particularly, to light-weight, metal-matrix composites, including uniformly distributed ceramic particles which increase the mechanical properties of the composite without significantly reducing its ductility and machinability.

### BACKGROUND OF THE INVENTION

Metal matrix composites (MMCs) are metals or alloys strengthened with tiny inclusions of another material which inhibit crack growth, and increase performance. MMCs have mechanical properties that are superior to those of most pure metals, some alloys, and most polymer-matrix composites, especially at high temperatures. The ability to tailor both mechanical and physical characteristics of MMCs is a unique and important feature of these materials.

Although the technology is relatively young, there are a number of significant applications, most notably, the space shuttle fuselage struts, space telescope boom-waveguides, and diesel engine pistons. In the future, metal-matrix composites are expected to become an important class of materials in numerous other commercial applications.

Although many metal-matrix composites having widely different properties exist, some general advantages of these materials over competing materials can be cited. MMCs are known to have higher strength-to-density ratios and higher stiffness-to-density ratios with better fatigue resistance than most unreinforced metals and some polymer matrix composites.

Numerous combinations of matrixes and reinforcements have been attempted since work on metal matrix composites began in the late 1950's. The most important matrix materials have been aluminum, titanium, magnesium, copper, and superalloys. Particular metal matrix composites that have been employed in the art have included aluminum matrixes containing boron, silicon carbide, alumina, or graphite in continuous fiber, discontinuous fiber, whisker, or particulate form. Magnesium, titanium, and copper have also been used as matrix metals with similar ceramic inclusions. Additionally, superalloy matrixes have been impregnated with tungsten wires to provide greater creep resistance at extremely high temperatures, such as those found in jet turbine engines.

Fabrication methods are an important part of the design process for MMCs. Considerable work is underway in this critical area, and significant improvements in existing processes appear likely. Current methods can be divided into two major categories: primary and secondary fabrication methods. Primary fabrication methods are used to create the metal matrix composite from its constituents. The resulting material may be in the form that is close to the desired final configuration, or it may require considerable additional processing, called secondary fabrication. Some of the more popular secondary fabrication methods include forming, rolling, metallurgical bonding, and machining.

One of the more successful techniques for producing MMCs, first suggested by Toyota for making pistons in 1983, is by infiltrating liquid metal into a fabric or prearranged fibrous configuration called a preform. Frequently, ceramic and/or organic binder materials are used to hold the fibers in position. The organic materials are then burned off before or during metal infiltration, which can be conducted under a vacuum, positive pressure, or both. One commonly employed pressure infiltration technique, which is known to reduce porosity in the final composite, is referred to as squeeze-casting.

The squeeze-casting process usually consists of placing a fiber or whisker preform in a cavity of a die, adding molten metal, and infiltrating the preform with the metal by closing the die and applying high pressure with a piston. The process is typically used for near net shaped parts of small dimensions. See Siba P. Ray and David I. Yun, "Squeeze-Cast Al₂O₃/Al Ceramic-Metal Composites", Ceramic Bulletin, Vol. 70, No. 2 (1991).

Although Ray and Yun suggest that ceramic matrix composites can be manufactured using preforms composed of alumina particles of .2 micron average particle size and including 14 to 48% open pores, this disclosure is limited to the production of ceramic-matrix composites (CMCs) having severely limited toughness, ductility, and machinability. Their set-up requires the use of expensive, heavy-walled dies and presses designed to withstand large pressure differentials, such as a 1,500-ton press.

It is also known to produce metal matrix composites by squeeze-casting followed by a secondary fabrication procedure, as suggested by Njishida et at., U.S. Patent No. 4,587,707. In this process, squeeze-casting is used to infiltrate a porous shaped article of ceramic particles with a molten metal, which is then permitted to solidify. High pressures of 50.5 to 101.3 MPa (500 to 1,000 atmospheres (15,000 to 150,000 psi)) were believed to be required for complete infiltration. The ceramic particles are provided by slender rods and are not uniformly distributed in the matrix. Since these concentrated layers of ceramic in the metal matrix are not intended to be present in the final product, mechanical forming is used to break up the rods into smaller pieces and distribute them throughout the matrix. The suggested rolling or extrusion techniques help to spread the now broken ceramic preforms more randomly throughout the composite; however, the result is far from a uniform distribution on a microscopic scale. Since the sintered ceramic rods are likely to be fractured in a nonuniform manner during the mechanical forming step, the resulting composite may contain concentrated, or agglomerated ceramic regions, which could limit the resulting composite's properties.

To alleviate the need for large pressure requirements, most known metal infiltration procedures use large particulate ceramics, greater than about 1 micron. Molten metal infiltration has not been considered a practical process for making metal-matrix composites incorporating submicron ceramic particles because the press size and pressure needs would be excessive and unrealistic. See Christodoulou et al., U.S. Patent No. 4,916,030, Col. 2, lines 25-38.

In order to dispense with the limitations and expense of large multi-ton presses, others have employed inert gas pressure metal infiltration techniques with loose ceramic powders. See Jingyu Yang and D.D.L. Chung, "Casting Particulate and Fibrous Metal-Matrix Composites by Vacuum Infiltration of a Liquid Metal Under an Inert Gas Pressure," Journal of Materials Science, Vol. 24, p.p. 3605-3612 (1989). Yang and Chung have developed a low pressure (6.895 to 17.24 MPa) (1,000 to 2,500 psi) molten metal infiltration technique that employs pressurized inert gas for forcing molten metal into loose ceramic fibers or particles. Particles ranging in size from .05 to 5 microns are used. By limiting the particles to a specific size range, this reference teaches that greater porosity in the close-packed particles can be provided, since the gaps between the particles are not filled by significantly smaller particles. It is this porosity volume fraction that is relied upon to permit the low pressure force to cause the molten liquid to infiltrate the loose layers of ceramic particles. Unfortunately, since the particles are loose and not sintered, they tend to agglomerate and randomly orient themselves during metal infiltration. This results in a relatively non-uniform distribution of particles throughout the matrix. Despite the expedient of using less pressure, therefore, the composite produced by infiltrating loose particles fails to achieve its full ductility and strength.

Metal-matrix composites are not without other well recognized drawbacks. The ceramic inclusions used to strengthen these composites are extremely hard, and are difficult to machine using conventional techniques. This results in serious tool-wear problems when the composite is machined into its final configuration. In some cases, the tool-wear becomes such a serious problem, that manufacturers resort to near-net shape manufacturing techniques, such as die casting and squeeze-casting, and the like, where machining is kept to a minimum, or is eliminated altogether. As reported in Charles T. Lane's "Machining Characteristics of Particulate-Reinforced Aluminum", Fabrication of Particulates Reinforced Metal Composites, Proceedings of an International Conference, Montreal, Quebec, Canada, ASM International, pp. 195-201 (1990), aluminum alloys reinforced with 10 to 15 micron ceramic particles wore through high-speed steel (HSS) tools in a matter of seconds, and dulled conventional and coated carbides in a matter of a few minutes. This paper reported that the only cost-efficient machining technique for MMCs was to use polyaystalline diamond (PCD) tools at speeds of up to 2,438 meters per minute. Other artisans have had similar experiences with machining MMCs, which has obviously limited their full commercial implementation.

K. Shanker et al., *Composites,* Vol 23, No. 1, January 1992, pp. 47-53 and US 5 196 273 A disclose TaC/metal matrix composites, wherein the metal is aluminum or copper. Aluminum is infiltrated into the TaC preform under argon at a temperature of 1300 - 1900 °C and a pressure of 0.1 MPa and reacts with the TaC. Copper has to be infiltrated in vacuum of < 100 Pa at a temperature of 1500 °C and yields two continuous matrices, one ductile (Cu) and one brittle (TaC). A milling step in preparing the TaC preform is not mentioned.

T. Hanamura et al., *Mat. Res. Soc. Symp. Proc.* Vol. 364, 1995, pp. 775-780 disclose γ TiAl-based alloy sheets containing Al₂O₃ particles, produced by a combination of vacuum induction melting and direct sheet casting. The aluminum content of the alloy is 3 at%.

The article by Michael S. Nagorka et al., *Metallurgical and Materials Transactions A, Physical Metallurgy and Materials Science* 26A (1995) April, No. 4, pp. relates to oxide dispersion strengthening of copper alloys. Cu-Zr and Cu-Y alloys were internally oxidized to yield ca. 1 vol% of ZrO₂ or Y₂O₃.

M. Otsuka et al, *The 33*^{*rd*} *Japan Congress of Materials Research,* March 1990, pp. 13-18 describe certain mechanically alloyed oxide dispersion strenghtened alloys which contain 0.27 mass% Y₂O₃.

Accordingly, there is a need for further process developments for manufacturing metal-matrix composites which have superior strength and uniformity, but which are also easy to machine and manufacture. There also remains a need for economically producing metal-ceramic composites without expensive heavy press machinery, or complicated processing techniques.

### SUMMARY OF THE INVENTION

This invention provides a metal-matrix composite and methods for the manufacture of metal matrix composites. The methods of this invention include providing a ceramic preform containing ceramic particles of average particle size no greater than about 3 microns. These tiny ceramic particles are distributed uniformly throughout the preform and are sintered to one another so that at least about one half of the volume of the preform is occupied by porosity. The method next includes the steps of placing the ceramic preform into a mold and contacting it with a molten metal. The molten metal is then forced into the preform so as to penetrate therethrough and occupy the pores. Finally, the molten metal is solidified to form a solid metal-matrix composite. In an important aspect of this invention, the resulting composite is machineable, and preferably, can be machined with a high-speed steel (HSS) tool bit for greater than about 1 minute without excessive wear to the bit.

Accordingly, this invention combines the high strength, stiffness, and wear resistance of ceramics with the machinability, toughness, and formability of metals. A small characteristic reinforcement size of less than about 3 microns, and preferably less than about 1 micron, in conjunction with a large volume fraction of porosity and a substantially uniform distribution of ceramic particles in a sintered preform are all employed to provide these composites. The composites of this invention provide improved room and elevated temperature strengths, increased modulus, and, unexpectedly, excellent machinability and ductility, even at high. ceramic loadings. These composites have been machined using only high-speed steel (HSS) milling, drilling, and tapping tooling without experiencing any difficulty. Excellent surface finishes were produced.

The MMCs of this invention exhibit high strength at room and elevated temperatures, since the small reinforcement size and interparticle spacing meets the criteria for dispersion strengthening. The small uniformly distributed ceramic particles permit the composite to behave much more like a metal than a typical MMC, permitting their use in applications requiring greater ductility, toughness, and formability. The particular metal infusion procedures of this invention are adaptable to multiple alloy and ceramic pairings and permit greater latitude for increasing the tensile modulus, as loadings approach 50 vol.%. Specific reinforcement ceramics and volume fractions can be selected which will permit designable engineered properties dictated by the application, including high elastic modulus, strength, and ductility.

In more preferred embodiments of this invention, other critical parameters are suggested, including preform porosities within the range of about 50 to 80 vol. %, a minimum preform compressive strength of about 3.45 MPa (500 psi), and the selection of preferred ceramic and metal alloy combinations for providing light-weight, high modulus composites. In the preferred manufacturing aspects of this invention, very low gas pressures can be used instead of a piston, to permit greatly facilitated processing of these composites without large capital expenditures. These processes can produce both bulk billets and near-net shape articles made from submicron sized particles by using pressures of less than about 20.68 MPa (3,000 psi). These processes are therefore inexpensive, and employ readily-available raw materials and otherwise standard liquid metal infusion techniques. All of these expedients can be accomplished by using a very uniform distribution of small reinforcement ceramics in a preform having readily infiltrated porosity.

### BRIEF DESCRIPTION OF THE DRAWINGS

FIG. 1: is a photomicrograph taken at 35,000 X magnification of an alumina-reinforced aluminum matrix composite manufactured by the preferred liquid metal infiltration techniques disclosed herein.

### DETAILED DESCRIPTION OF THE INVENTION

Machinable metal-matrix composites are provided by this invention which are derived from combining ceramic particles of no greater than about 3 microns with molten metal in an extremely uniform manner. By employing smaller ceramic particles, preferably of submicron size, and distributing them throughout a metal-matrix so as to avoid agglomeration, both high ductility and strength can be provided to the composite without limiting machinability. In preferred embodiments of this composite, at least 80% of the ceramic particles are uniformly distributed on a scale of three times the particle size, and more preferably, at least 90% of the ceramic particles are uniformly distributed on a scale of twice the particle size. This degree of fine particle distribution virtually eliminates large inclusions and agglomerations which detract from the ductility, strength, and machinability of the composites.

Although this invention relates to all types of metal-ceramic composites, including ceramic-matrix composites (CMCs), it is particularly applicable to metal-matrix composites (MMCs) having a larger volume fraction of metal than ceramic. These MMCs can be made from many different combinations of matrix material and reinforcing particles to develop whatever special set of properties is required for each application.

This invention contemplates employing ultra-high strength metal matrixes including those having a yield strength of about 70 to 2,000 MPa. Such metals include, for example, cobalt and its alloys, martensitic stainless steels, nickel and its alloys, and low-alloy hardening steels. High strength metals and alloys are also potential candidates for the matrixes of this invention, including tungsten, molybdenum and its alloys, titanium and its alloys, copper casting alloys, bronzes, coppers, niobium and its alloys, and superalloys containing nickel, cobalt, and iron. Medium strength metals and alloys can also be considered, including hafnium, austenitic stainless steels, brasses, aluminum alloys between 2,000 and 7,000 series, beryllium-rich alloys, depleted uranium, magnesium alloys, silver, zinc die casting alloys, coppers, copper nickels, copper-nickel-zincs, and other metals having a yield strength of about 40 to 690 MPa. Finally, this invention optionally employs low strength, low density alloys for the matrixes of this invention. Such metals are represented by gold, cast magnesium alloys, platinum, aluminum alloys of the 1,000 series, lead and its alloys, and tin and its alloys. These materials have a yield strength of only about 5 to 205 MPa. Most desirably, this invention employs light-weight metals and those which are relatively inexpensive and widely available, such as aluminum, lithium, beryllium, lead, tin, magnesium, titanium, and zinc, and metals which have superior electrical properties, such as copper, silver, and gold. All of these selections can be provided in commercially pure, or alloyed, form. Specific alloys which have been recognized to have particular usefulness in MMCs include Al-1 Mg-0.6 Si, Al-7 Si-1 Mg, Al-4.5 Cu, Al-7 Mg-2 Si, and Al-Fe-V-Si.

Although alloys and commercially pure metals can be employed to produce the matrixes of this invention, a pure metal is the matrix of choice, since ceramic dispersion strengthening is all that is required for improved properties. A pure metal also offers enhanced corrosion resistance over alloys, and eliminates the effects of overaging of precipitates. Pure metals also boost elevated temperature capability by increasing the homologous melting point over comparable alloys. Finally, pure metals eliminate the difficulties associated with microsegregation and macrosegregation of the alloying elements in non-eutectic alloys during solidification.

The ceramic or second phase constituents of the metal matrix composites of this invention are desirably of a size which does not interfere with machining by HSS tooling. It has been discovered that machinability can be preserved only if these ceramic particles are less than about 3 microns, although this invention preferably employs a size range of about 0.01 to .5 microns. The ceramic particles should be thermally and chemically stable for the time and temperature of the particle fabrication process and environmental conditions of service.

These ceramic particles should not decompose at high temperatures, nor react with the metal matrix. If they tend to diffuse into the matrix, diffusion of the reinforcement must be slow, so that the strength of the composite does not seriously degrade. Ultra-fine reinforcement particles having a volume fraction of about 20 to 40% are particularly advantageous in yielding composites with improved Young's modulus, ductility, and machinability.

Exemplary second phase ceramic candidates include borides, carbides, oxides, nitrides, silicates, sulfides, and oxysulfides of elements which are reactive to form ceramics, including, but not limited to, transition elements of the third to sixth groups of the Periodic Table. Particularly useful ceramic-forming or intermetallic compound-forming constituents include aluminum, titanium, silicon, boron, molybdenum, tungsten, niobium, vanadium, zirconium, chromium, hafnium, yttrium, cobalt, nickel, iron, magnesium, tantalum, thorium, scandalum, lanthanum, and the rare earth elements. More exotic ceramic materials include titanium diboride, titanium carbide, zirconium diboride, zirconium disilcide, and titanium nitride.

Carbon-based ceramics can also be useful as the ceramic phase, including natural and synthetic diamonds, graphite, fullerenes, diamond-like graphite, etc. Certain ceramics, because of their availability, ease of manufacture, low cost, or exceptional strength-inducing properties, are most desirable. These include Al₂O₃, SiC, B₄C, MgO, Y₂O₃, TiC, graphite, diamond, SiO₂, ThO₂, and TiO₂. These ceramic particles desirably have an aspect ratio of no greater than about 3:1, and preferably no greater than about 2:1, but can be represented by fibers, particles, beads, and flakes, for example. However, particles are preferred for machinability.

Alternatively, the ceramic reinforcements of this invention can have aspect ratios ranging from equiaxed, to platelets and spheredized configurations. The particle size distribution can range from mono-sized, to a gausean distribution, or a distribution having a wide tail at fine sizes. These particles can be mixed using a variety of wet and dry techniques, including ball milling and air abrasion.

The preferred binders employed in connection with the ceramic reinforcements can include: inorganic colloidal and organic binders, such as, sintering binders, low temperature (QPAC), and high temperature colloidal binders. Such binders have included polyvinyl alcohol, methyl cellulose, colloidal alumina, and graphite.

Metal-matrix composites made in accordance with this invention and containing one or more of the above metals, alloys, and ceramic particles, can be fabricated into many useful configurations for a variety of applications. Some of the more interesting applications appear below in TABLE I.

**TABLE I:**

| **Representative Metal-Ceramic Composites and Potential Applications** | | |
|---|---|---|
| Matrix | Fiber | Potential Applications |
| Aluminum | Graphite | Satellite, missile, and helicopter structures |
| Magnesium | Graphite | Space and satellite structures |
| Lead | Graphite | Storage-battery plates |
| Copper | Graphite | Electrical contacts and bearings |
| Aluminum | Boron | Compressor blades and structural supports |
| Magnesium | Boron | Antenna structures |
| Titanium | Boron | Jet-engine fan blades |
| Aluminum | Borsic | Jet-engine fan blades |
| Titanium | Borsic | High-temperature structures and fan blades |
| Aluminum reactors | Alumina | Superconductor restraints in fusion-power |
| Lead | Alumina | Storage-battery plates |
| Magnesium | Alumina | Helicopter-transmission structures |
| Aluminum | SiC | High-temperature structures |
| Titanium | SiC | High-temperature structures |
| Superalloy (Co-base) | SiC | High-temperature engine components |
| Superalloy | Molybdenum | High-temperature engine components |
| Superalloy | Tungsten | High-temperature engine components |

The performance of the resulting composites of this invention is intimately linked to the uniformity of the preform used in the preferred metal infiltration procedures. These preforms can be made by a variety of procedures including sediment casting, injection molding, gel casting, slip casting, isopressing, ultrasonic techniques, filtering, extruding, pressing, and the like. Preferably, colloidal processing is employed to make the preforms. Volatile additions and controlled agglomeration of the slurries can be used to adjust particle volume fraction within the desired ranges.

Following the preparation of a green preform, the preform is preferably dried, or fired. This can be accomplished by microwave processing, freeze drying, or air/inert gas firing. Test bars can also be prepared along with the preform so that a determination of the modulus of rupture, or tensile properties, can be evaluated prior to pressure infiltration. A target compressive strength of at least about 3.45 MPa (500 psi), and preferably about 4.83 to 8.274 MPa (700 to 1,200 psi), is desirable for the sintered preform.

The preforms of this invention are ideally pressure infiltrated with liquid metal to produce billets or shaped articles. Pressure infiltration can include all types of liquid metal infiltration (LMI) processes, including: inert gas pressure techniques, squeeze casting, and die casting, etc. In a most preferred procedure, inert gas pressure infiltration is employed. This technique includes the key steps of: evacuation of the preform prior to infiltration, adequate pressure control for infiltration without preform disruption, and directional solidification under pressure to feed solidification shrinkage.

In a mass production environment, fabrication of large-sized billets could be followed by wrought processing to common product forms. Pressure infiltration coupled with wrought processing offers a potential of low cost, high performance composite manufacturing for a wide variety of structural applications. Wrought processing can include such procedures as: extrusion, rolling, forging, etc. Net shape processing can also be employed, including: die casting and squeeze casting. In these latter procedures, large billets, due to the inherent stability of the claimed composites, can be remelted and processed in the liquid state to produce near net shape components. Approximate properties for an aluminum and magnesium matrix MMC prepared by the preferred processes of this invention are included below in TABLE II.

**TABLE II:**

| **Approximate Physical Properties of Dispersion Strengthened Aluminum and Magnesium** | | |
|---|---|---|
| | Aluminum 25% Alumina | Magnesium* 20% Diamond |
| Density | 3.00 g/cc | 2.00 g/cc |
| Tensile Strength | 413 MPa (60 ksi) | 379 MPa (55 ksi) |
| Vickers Hardness | 120 MPa | 110 MPa |
| Young's Modulus | 124 Pa (18 msi) | 151 Pa (22 msi) |

| | | |
|---|---|---|
| *Proposed example | | |

Applicants have evaluated the preferred loading ranges for the MMCs of this invention, and have determined that a 15 vol. % ceramic loading improves the modulus of commercially pure aluminum and magnesium by about 30%. A 25 vol. % of ceramic particles improves the modulus by about 50 to 60%, and a 55 vol.% ceramic loading improves the modulus by about 100%, but ductility begins to suffer. Ceramic loadings of up to 45 vol. % produced MMCs which were machined with high speed steel without significant wear. It was further noted that when ceramic particles exceeded about 3 microns, the machinability of the MMC decreased dramatically. With respect to the volume fraction, it was further noted that ceramic loadings greater than about 50% significantly lowered the ductility of the composite, and loadings significantly below 15 vol. % produced no significant modulus boost. Lower loadings were also very difficult to infiltrate, since the preforms were too weak to sustain infiltration pressures without disruption.

The present invention will be further described with reference to the following examples.

### Example I

A composite material was prepared having a commercially pure Al matrix including 25 vol. % Al₂O₃, about .2 micron average particle size on a population basis. As a preliminary step, the raw materials were weighed out as follows:
Reinforcement: A-16SG, calcined Al₂O₃, Alcoa Industrial Chemical Division, 259.8 grams.
Carrier: POLAR distilled water, Polar Water Company, 1205.8 grams.
Filler: Micro 450 (M-450) graphite, Asbury Graphite Mills, Inc., 184.6 grams
Colloidal Binder: Inorganic NYACOL, AL2O, high temperature coating/binder, Nyacol Products, Inc., 86.0 grams.

This mixture was combined in a mill using the following mill parameters: slurry solids content of 10% and mill fill level of 30%. The slurry batch was milled for about 23 to 25 hours, removed from the mill, and disposed in a pressure filtration unit. The slurry was filtrated at 2.41 MPa (350 psi) for about 36 to 60 hours. When filtration was complete, the green preform was removed from the filtration unit. It was measured to have dimensions of about 4.9 cm in diameter X 12 cm long. The green preform had a reinforcement loading of about 22 vol. %. The green preform was then dried at ambient conditions until a weight loss of at least about 25 wt.% had been achieved. This took about five days.

The dry preform was then placed in a furnace and fired according to the following schedule:

| Ramp Seq. | Ramp Rate (°C/hr) | Ramp Time (hr) | Hold Temp (°C) | Hold Time (hr) |
|---|---|---|---|---|
| 1/2 | 25 | 14 | 325 | 2 |
| 3/4 | 50 | 12 | 900 | 30 |
| 5/6 | 50 | 6 | 1,200 | 1.5 |
| 7/8 | 100 | 12 | 22 | 24 |

The fired preform had a loading of about 25 vol. % of sintered ceramic particles. It was removed and inspected, and a weight loss of about 40 wt.% was noted. This weight loss insured that all filler material had been removed. A mild steel infiltration crucible was then prepared by coating with a graphite wash coating DAG 154 Graphite Lubricating/Resistance Coating, available from Achesion Colloids Company. The interior of the crucible was then lined with GRAFOIL graphite paper, Grade GTB available from UCAR Carbon Company, Inc. The fired preform was then inserted into the lined crucible and a preform support rod was inserted to prevent floating. The crucible was then inserted into the pressure infiltration unit, which was custom built. The pressure infiltration unit was evacuated, and then preheated using the following heat cycle:

| Ramp Seq. | Ramp Time (hr) | Hold Temp (°C) | Hold Time (hr) |
|---|---|---|---|
| 1/2 | 2 | 200 | 0:05 |
| 3/4 | 8 | 700 | 2 |

Approximately 650 grams of commercially pure aluminum (99.9% aluminum, 2 to 5 shot available from Alcoa) was then melted in an electrical resistance furnace and covered with Flux No. 770 Cover Flux, available from Asbury Graphite Inc. The infiltration unit was then backfilled with argon, the crucible was removed from the pressure infiltration unit, and the molten alloy was poured into the crucible. The crucible was then placed into the pressure infiltration unit, and it was again evacuated. After evacuation, the unit was pressurized with argon to about 14.8 MPa (2,150 psi) in about 40 to 80 seconds and held for five minutes. The unit was then vented, and the crucible was placed onto a water-cooled chill at the bottom of the pressure infiltration unit. The unit was once again repressurized to 6.895 MPa (1,000 psi) for solidification. The mixture was permitted to cool for about one hour until directionally solidified. The sample was removed from the pressure infiltration unit, the crucible was cut off, and the alloy head was removed.

Under a scanning electron microscope, a fracture surface of one sample of the above composite was visually inspected at 35,000 X. The micrograph is shown in FIG. 1. The observed particle size was found to be about .05 to .4 microns, with .2 microns being typical, and an interparticle spacing of about .05 to .4 microns was measured.

The following mechanical properties were measured after two samples were removed from the resulting billet:
Yield Strength MPa (ksi) = 170.3 (24.7)
Ultimate Tensile Strength MPa (ksi) = 331 (48.0)
% Elongation = 6.0
1.00 - SR, Short Rod Fracture Toughness = 18.1 MN·m^{-3/2} (16.5 KSi(IN)²)

Others samples were extruded at 440°C (825°F) and further samples were prepared for hardness, tensile and fatigue properties, with the following results:

| Hardness | |
|---|---|
| As extruded | Rb 57 |
| As solutionized (940 F/1 hr/WQ) | Rb 59 |
| Solutionized (940 F/1 hr/WQ) plus Age (400 F/2 hr/AC) | Rb 56 |

| Hot Hardness | | |
|---|---|---|
| Temperature, °C (°F) | Load, Kg | BHN |
| RT | 750 | 103 |
| RT | 500 | 99.3 |
| 149 (300) | 500 | 68.7 |
| 260 (500) | 500 | 46.1 |
| 315 (600) | 500 | 41.6* |

| | | |
|---|---|---|
| *Indentor bottomed | | |

| Tensile Properties | | | |
|---|---|---|---|
| Property | RT | 149°C (300°F) | 260°C (500°F) |
| UTS MPa (KSI) | 344 (49.9) | 245 (35.6) | 170 (24.7) |
| YS MPa (KSI) | 203 (29.5) | 189 (27.5) | 158 (22.9) |
| % El. | 11 | 11 | 12 |
| % RofA | 17 | 17 | 15.5 |

| Smooth Fatigue | | |
|---|---|---|
| Stress, KSI | Temperature, °C (°F) | Cycles to Failure X 10E6 |
| 20 | 260 (500) | 0.335 |
| 15 | 260 (500) | 0.690 |
| 10 | 260 (500) | 187.5 |

### Example II

A composite material was prepared using an Al-2.SMg matrix having 25 vol. % fraction Al₂O₃ particles, about .2 micron average particle size on a population basis using the same procedure as described in Example I, except the matrix included 5052-H32 Al-2.5Mg alloy, in the form of a 0.249 cm X 48 cm X 24 cm plate. The process parameters were identical, except the Al-2.5Mg alloy was substituted for the commercially pure aluminum. No cover flux was used during melting of the alloy, and the hold temperature during infiltration was about 695°C. The following properties were obtained using some of the same testing procedures as disclosed in Example I:
Sonic Modulus Pa (MSI) = 109.3 Pa (15.85)
Poisons Ratio = 0.318
Density (g/cm³) = 3.023

| Test Temp °C (F) | Uniform Elongation % | Plastic Elongation % | U.T.S. MPa (KSI) | YS MPa (KSI) |
|---|---|---|---|---|
| 25 (77) | 6.33 | 6.514 | 389.4 (56.47) | 321.7 (46.66) |
| 93.3 (200) | 5.20 | 8.68 | 335.4 (48.64) | 265.0 (38.43) |
| 149 (300) | 4.78 | 16.2 | 274.2 (39.77) | 70.40 (10.21) |
| 25 (77*) | 3.92 | 3.948 | 392.6 (56.94) | 321.7 (46.66) |

| | | | | |
|---|---|---|---|---|
| *Tested after 149°C (300°F)/100 hrs exposure | | | | |

### Example III

A composite material was prepared which included a commercially pure Al matrix including 40 vol. % Al₂O₃, .2 micron average particle size on a population basis. The raw materials of Example I were the same except for the fact that an organic binder, AIRVOL 540, polyvinyl alcohol, from Chemicals Group Sales of Air Products and Chemical, Inc. was employed, and a colloidal chemistry adjustment was made which included the addition of nitric acid, 69.0 to 71.0%, BAKER ANALYZED Reagent, HNO₃, from VWR Scientific. As with previous examples, the dried ingredients were weighed out as follows:
Reinforcement: A-16 SG calcined Al₂O₃, 633.0 grams.
Carrier: POLAR Distilled Water, 920.7 grams.
Filler: Micro 450 (M-450) graphite, 104.5 grams.
Organic Binder: (6 wt. % solution in water), AIRVOL 540, 30.1 grams.
Colloidal Chemistry Adjuster: nitric acid, 0.4 ml.

This mixture was combined in a similar milling procedure as was used in Example I with the following mill parameters: slurry solids content of 17.5% and mill fill level of 25%. The slurry batch was milled for about 23 to 25 hours, removed from the mill, and disposed in a pressure filtration unit.

The slurry was filtrated at 350 psi for about 20 to 30 hours. When filtration was complete, the green preform, 37 vol. % ceramic, was removed from the filtration unit. It was measured to have dimensions of 4.9 cm in diameter X 14 cm long. The green preform was then dried at ambient conditions until a weight loss of at least 23 wt. % had been achieved. This took about five days.

The dried preform was then placed in a furnace and fired according to the following schedule:

| Ramp Seq. | Ramp Rate (°C/hr) | Ramp Time (hr) | Hold Temp (°C) | Hold Time (hr) |
|---|---|---|---|---|
| 1/2 | 25 | 14 | 325 | 2 |
| 3/4 | 50 | 12 | 900 | 30 |
| 5/6 | 50 | 4 | 1,100 | 2 |
| 7/8 | 100 | 11 | 22 | 24 |

The fired preform had a loading of about 40 vol. % of sintered ceramic particles. It was removed and inspected, and a weight loss in excess of about 15 wt. % was noted.

A mild steel infiltration crucible was then prepared, inserted into the infiltration unit and evacuated in accordance with substantially the same procedure as described for Example I. The unit was thereafter preheated using the following heat cycle:

| Ramp Seq. | Ramp Time (hr) | Hold Temp (°C) | Hold Time (hr) |
|---|---|---|---|
| 1/2 | 2 | 200 | 0:05 |
| 3/4 | 8 | 700 | 2 |

Approximately 600 grams of commercially pure aluminum, as used above in Example I, was then melted, and inert gas infiltration was used to prepare a composite substantially in accordance with the procedures of Example I.

The following mechanical properties were measured:
Material Condition: As Cast
   Sonic Modulus Pa (MSI) = 122 (17.7)
   Poisons Ratio = 0.288
   Density (g/cm³) -3.113
Material Condition: Extruded
   Ultimate Tensile Strength MPa (ksi) = 448 (65)
   Elongation = 4%

### Hardness

70 Rb

### Example IV

A composite material was prepared having a commercially pure Mg matrix including 30 vol. % MgO ceramic particles, about .8 micron average particle size (about .2 micron after milling). The raw materials employed were the same as those used in Example I with the following exceptions: the reinforcement included MAGCHEM 20-M, technical grade magnesium oxide from Martin Marietta Magnesia Specialties, Inc.; the carrier employed was denatured ethanol from E.K. Industries, Inc.; the organic binder was Bulls Eye Shellac, Clear Sealer and Finish, from Williams Zinsser & Co., Inc., and the matrix consisted of commercially pure magnesium, 99.8 wt. % magnesium 0.453kg, (1 pound) sticks, 3.3cm (1.3 inch)diameter X 30cm (12 inch) in length.

The raw materials were weighted out as follows:
Reinforcement: MAGCHEM 20-M magnesium oxide, Martin Marietta Magnesia Specialties, Inc., 232.3 grams.
Carrier: POLAR Distilled Water, 727.2 grams.
Filler: Micro 450 (M-450) graphite, 89.6 grams.
Organic Binder: Bulls Eye Shellac, 116.4 grams.

This mixture was combined in a mill using the following mill parameters: slurry solids content of 10% and mill fill level of 25%.

The slurry batch was milled according to the milling procedures of Example I. When filtration was complete, the green preform was removed from the filtration unit. It was measured to have dimensions of about 4.9 cm diameter X 10 cm long. The green preform had a reinforcement loading of about 26 vol. %, and was then dried at ambient conditions until a weight loss of at least about 25 wt.% had been achieved. This took about five days.

The dried preform was then placed in a furnace and fired according to the following schedule:

| Ramp Seq. | Ramp Rate (°C/hr) | Ramp Time (hr) | Hold Temp (°C) | Hold Time (hr) |
|---|---|---|---|---|
| 1/2 | 25 | 14 | 325 | 6 |
| 3/4 | 50 | 14 | 700 | 30 |
| 5/6 | 50 | 4 | 1,100 | 1 |
| 7/8 | 100 | 12 | 22 | 24 |

The fired preform had a loading of about 29 vol.% of sintered ceramic particles. It was removed and inspected, and a weight loss of at least about 34 wt. % was noted.

An infiltration crucible was prepared and set up substantially as described for Example I. Approximately 300 grams of matrix magnesium alloy was deposited on the top of the preform and preform support rod. The crucible was inserted into the pressure infiltration unit, the unit was evacuated and backfilled to an argon pressure of about 300 psi. The unit was then preheated using the following heat cycle:

| Ramp Seq. | Ramp Time (hr) | Hold Temp (°C) | Hold Time (hr) |
|---|---|---|---|
| 1/2 | 2 | 200 | 0:05 |
| 3/4 | 8 | 705 | 2 |

After the two-hour hold at about 705°C, the unit was evacuated. Alter evacuation, it was pressurized with argon to about 14.82 MPa (2,150 psi) and held for five minutes. The directional solidification and removal steps were substantially the same as those described above for Example I. Samples were prepared and a hardness value of 65 Rb was measured. Hot hardness values substantially paralleled the trend for the aluminum-matrix samples.

### Machinability Test

Samples were prepared from the Al/25 vol.% Al₂O₃ (Example I); Al/40 vol.% Al₂O₃ (Example II); Al-2.5Mg/25 vol.% Al₂O₃ (Example III); and Mg/30 vol. % MgO (Example IV).

Each of the samples was subjected to the following machining operations with the noted results:
Face milling and end milling was preformed with HSS tooling. No difficulty was experienced using approximately 0.66 m/sec (130 sfm) speeds and up to about 0.63 cm (1/4 inch) roughing cuts. The surface finish was good.

Drilling was performed with uncoated regular-twist HSS drills without problems. The drill was operated at about 0.51m/sec (100 sfm). Drilling holes from about 0.85mm (1/32 inch) diameter up to about 1.59cm (5/8 inch) diameter were made with no apparent limitation in the depth.

Tapping was performed with an uncoated 3 flute HSS tap, tapped by hand to sizes ranging from about 0.52cm (1/8 inch) to about 1.9cm (3/4 inch)course and fine threads. No difficulty was encountered.

Samples prepared from the Al/25 vol. % Al₂O₃ and Al2.5 vol. % Mg/25 vol. % Al₂O₃ were turned on a lathe at about 1.78 m/sec (350 sfm) using a solid carbide tool bit. The tool bit removed at least 98.3 cm³ (6 cubic inches) of material and operated for at least three hours without difficulty.

An Al/40 vol. % Al₂O₃ sample was turned on a lathe at about 1.78 m/sec (350 sfm)using a HSS tool bit. The tool bit removed at least about 49.2 cm³ (3 cubic inches) of material and operated for at least two hours without difficulty. Good to excellent surface finishes were obtained.

### Comparative Example V

Drilling was performed using a 356-T6 Al-matrix reinforced with 20 vol. % SiC (10 to 15 micron average particle size), (DURALCAN F3A.20S). The drilling operation was preformed with a 0.63cm (1/4 inch)HSS drill bit using a hand drill. The drill bit penetrated about 0.63cm (1/4 inches) and was dulled to the point where it required sharpening to be used again.

An attempt was made to cut this material using a band saw. The saw penetrated about 0.63cm (1/4 inches) and then stopped. Both of these hand drilling and band saw techniques were later duplicated on an Al/25 vol. % Al₂O₃ sample of Example I without difficulty.

### Comparative Example VI

An additional comparative sample was prepared by gas pressure infiltration of loose ceramic powder of 10 micron average particle size SiC and commercially pure Mg liquid metal. The resulting Mg/40 to 45 vol. % SiC composite was turned on a lathe using a solid carbide tool bit. The lathe cut for only a few seconds, when the bit began to dull and merely push the material.

### Comparative Example VII

A further comparative sample was prepared using the same technique as described for Example VI with 3 micron average particle size SiC. An attempt was made to band saw the resulting Mg/40 to 45 vol.% SiC composite. The band saw quickly stopped in about 10 to 15 seconds without significant penetration into the matrix.

From the foregoing, it can be realized that this invention provides machinable, high modulus metal-matrix composites and metal infiltration techniques for preparing these composites. Critical parameters have been discovered which map the necessary ranges of volume fraction of porosity and particle size distribution necessary for low pressure metal infiltration and optimum mechanical properties. Although various embodiments have been illustrated, this was for the purpose of describing and not limiting the invention. Various modifications, which will become apparent to one skilled in the art, are within the scope of this invention described in the attached claims.

## Claims

1. A method for manufacturing a metal-matrix composite comprising the steps of:
providing a ceramic preform having submicron ceramic particles and sintering the ceramic particles to one another;
disposing of said ceramic preform into a mold;
contacting said ceramic preform with a molten metal;
causing said molten metal to penetrate into said preform; and
permitting said molten metal to solidify to form a metal matrix composite;
wherein said metal-matrix composite is machinable with a high speed steel bit,
**characterised in that**
in a first step a colloidal slurry of ceramic particles in a liquid is subjected to a milling step to provide the colloidal slurry of ceramic particles wherein said particles have a particle size of no greater than 1 micron; and subsequently said ceramic particles are separated from the liquid to provide a ceramic preform having a uniform distribution of said submicron ceramic particles.

2. A method for manufacturing a metal-matrix composite in accordance with claim 1 wherein at least 80% of said ceramic particles are uniformly distributed on a scale of three times the average particle size.

3. A method for manufacturing a metal-matrix composite in accordance with claim 2 wherein at least 90% of the ceramic particles are uniformly distributed on a scale of twice the average particle size.

4. A method for manufacturing a metal-matrix composite in accordance with claim 1 wherein the step of causing said molten metal to penetrate into said preform is accomplished by pressure infiltration.

5. The method of claim 4 wherein said ceramic preform includes 50 to 85% porosity by volume.

6. The method of claim 5 wherein said ceramic preform consists of 60 to 80% porosity by volume.

7. The method of claim 4 wherein said composite comprises a tensile modulus which is at least 30 to 200% greater than the tensile modulus of said metal.

8. The method of claim 1 wherein said providing step of a ceramic preform comprises filtering, extruding, pressing or slip casting a precursor of said particles to produce a green preform.

9. The method of claim 1 wherein said causing step comprises molten metal infiltration, whereby said molten metal is forced into the pores of said preform by a pressurized gas.

10. The method of claim 9 wherein said pressurized gas has a pressure of 6.895 to 20.685 MPa (1,000 to 3,000 psi), and said preform has a compressive strength of at least 3.448 MPa (500 psi).

11. The method, of claim 1 wherein said molten metal is driven into said preform by pressure infiltration so as to cause said molten metal to penetrate into the pores of said preform without disrupting said preform.

12. The method of claim 11 wherein the ceramic particles comprise: an oxide, boride, nitride, carbide, carbon, silicide, sulfide, oxysulfide or a mixture thereof.

13. The method of claim 11 wherein the colloidal slurry of the ceramic particles is mixed with up to 70 vol.%, based upon the volume of dry ingredients, of a filler, binder or mixture thereof.

14. The method of claim 10 wherein said pressurized gas is an inert gas having a pressure of 10.34 MPa to 17.23 MPa (1,500 to 2,500 psi).

15. The method of claim 11 wherein said metal-matrix composite comprises a near net shape.

16. The method of claim 1, wherein said molten metal is selected from the group consisting of: Al, Li, Be, Pb, Ag, Au, Sn, Mg, Ti, Cu, Zn or a mixture thereof.

17. The method of claim 1 wherein said step of providing a preform comprises:
pressure filtrating a precursor of said ceramic particles with a graphite filter in the separation step, suspending said filtered particles with a graphite filler and
inorganic binder to form a green preform; and firing said green preform to remove said filler, whereby a portion of said ceramic particles are sintered to one another.

18. The method of claim 9 wherein said forcing step comprises evacuating a gas from said preform by an applied vacuum, and forcing said molten metal into the pores of said preform with a pressurized argon-containing gas.

19. The method of any of claims 1 to 18 wherein said particles are Al₂O₃ and said molten metal is Al.

20. The method of any of claims 1 to 19, wherein said particles have a particle size of from 0.01 to 0.5 microns.

21. A metal-matrix composite comprising a uniform distribution of alumina particles having an average particle size no greater than 1 micron and aluminum substantially uniformly distributed with said alumina particles, at least 80% of said alumina particles being uniformly distributed on a scale of three times the average particle size wherein the alumina ceramic loading is from 15 vol% to 50 vol.%.

## Patentansprüche

1. Verfahren zur Herstellung eines Metall-Matrix-Verbundstoffes, umfassend die Schritte:
Bereitstellen einer Keramik-Vorform mit Submikrometer-Keramikteilchen und Aneinandersintern der Keramikteilchen;
Anordnen der Keramik-Vorform in einer Form;
In-Kontakt-Bringen der Keramik-Vorform mit einem geschmolzenen Metall;
Bewirken, dass das geschmolzene Metall in die Vorform eindringt; und
Gestatten, dass sich das geschmolzene Metall verfestigt, um einen Metall-Matrix-Verbundstoff zu bilden;
wobei der Metall-Matrix-Verbundstoff mit einer Hochgeschwindigkeits-Stahl-Bohrerspitze maschinell bearbeitbar ist, **dadurch gekennzeichnet, dass**
in einem ersten Schritt eine kolloidale Aufschlämmung von Keramikteilchen in einer Flüssigkeit einem Mahlschritt unterzogen wird, um eine kolloidale Aufschlämmung von Keramikteilchen bereitzustellen, in der die Teilchen eine Teilchengröße von nicht mehr als 1 Mikrometer aufweisen; und anschließend die Keramikteilchen von der Flüssigkeit abgetrennt werden, um eine Keramik-Vorform mit einer gleichmäßigen Verteilung der Submikrometer-Keramikteilchen bereitzustellen.

2. Verfahren zur Herstellung eines Metall-Matrix-Verbundstoffes nach Anspruch 1, in dem mindestens 80% der Keramikteilchen gleichförmig auf einer Skala des Dreifachen der durchschnittlichen Teilchengröße verteilt sind.

3. Verfahren zur Herstellung eines Metall-Matrix-Verbundstoffes nach Anspruch 2, in dem mindestens 90% der Keramikteilchen gleichmäßig auf einer Skala des Zweifachen der durchschnittlichen Teilchengröße verteilt sind.

4. Verfahren zur Herstellung eines Metall-Matrix-Verbundstoffes nach Anspruch 1, in dem der Schritt des Bewirkens, dass das geschmolzene Metall in die Vorform eindringt, durch Druckinfiltration bewerkstelligt wird.

5. Verfahren nach Anspruch 4, in dem die Keramik-Vorform 50 bis 85% Porosität bezüglich Volumen einschließt.

6. Verfahren nach Anspruch 5, in dem die Keramik-Vorform aus 60 bis 80% Porosität bezüglich Volumen besteht.

7. Verfahren nach Anspruch 4, in dem der Verbundstoff einen Zugmodul umfasst, der mindestens 30 bis 200% größer als der Zugmodul des Metalls ist.

8. Verfahren nach Anspruch 1, in dem der Schritt des Bereitstellens einer Keramik-Vorform das Filtrieren, Extrudieren, Pressen oder Schlickergießen einer Vorstufe der Teilchen umfasst, um eine grüne Vorform zu erzeugen.

9. Verfahren nach Anspruch 1, in dem der Schritt des Bewirkens eine Infiltration von geschmolzenem Metall umfasst, wodurch das geschmolzene Metall durch ein unter Druck stehendes Gas in die Poren der Vorform hineingedrückt wird.

10. Verfahren nach Anspruch 9, in dem das unter Druck stehende Gas einen Druck von 6,895 bis 20,685 MPa (1000 bis 3000 psi) aufweist und die Vorform eine Druckfestigkeit von mindestens 3,448 MPa (500 psi) aufweist.

11. Verfahren nach Anspruch 1, in dem das geschmolzene Metall durch Druckinfiltration in die Vorform getrieben wird, um zu bewirken, dass das geschmolzene Metall in die Poren der Vorform eindringt, ohne die Vorform zu zerbrechen.

12. Verfahren nach Anspruch 11, in dem die Keramikteilchen: ein Oxid, Borid, Nitrid, Carbid, Kohlenstoff, ein Silicid, Sulfid, Oxysulfid oder eine Mischung derselben umfassen.

13. Verfahren nach Anspruch 11, in dem die kolloidale Aufschlämmung der Keramikteilchen mit bis zu 70 Vol.-%, bezogen auf das Volumen an trockenen Bestandteilen, eines Füllstoffes, Bindemittels oder einer Mischung derselben gemischt ist.

14. Verfahren nach Anspruch 10, in dem das unter Druck stehende Gas ein Inertgas mit einem Druck von 10,34 MPa bis 17,23 MPa (1500 bis 2500 psi) ist.

15. Verfahren nach Anspruch 11, in dem der Metall-Matrix-Verbundstoff eine angenäherte Netzform aufweist.

16. Verfahren nach Anspruch 1, in dem das geschmolzene Metall aus der Gruppe ausgewählt ist, die aus: Al, Li, Be, Pb, Ag, Au, Sn, Mg, Ti, Cu, Zn oder einer Mischung derselben besteht.

17. Verfahren nach Anspruch 1, in dem der Schritt der Bereitstellung einer Vorform umfasst: Druckfiltrieren einer Vorstufe der Keramikteilchen mit einem Graphit-Filter in dem Abtrennungsschritt, Suspendieren der filtrierten Teilchen mit einem Graphit-Füllstoff und einem anorganischen Bindemittel, um eine grüne Vorform zu bilden; und Brennen der grünen Vorform, um den Füllstoff zu entfernen, wodurch ein Teil der Keramikteilchen aneinandergesintert wird.

18. Verfahren nach Anspruch 9, in dem der Schritt des Hineindrückens das Evakuieren eines Gases aus der Vorform durch ein angelegtes Vakuum und das Hineindrücken des geschmolzenen Metalls in die Poren der Vorform mit einem unter Druck stehenden Argon-haltigen Gas umfasst.

19. Verfahren nach irgendeinem der Ansprüche 1 bis 18, in dem die Teilchen Al₂O₃ sind und das geschmolzene Metall Al ist.

20. Verfahren nach irgendeinem der Ansprüche 1 bis 19, in dem die Teilchen eine Teilchengröße von 0,01 bis 0,5 Mikrometer aufweisen.

21. Metall-Matrix-Verbundstoff, umfassend eine gleichmäßige Verteilung von Aluminiumoxid-Teilchen mit einer durchschnittlichen Teilchengröße von nicht mehr als 1 Mikrometer und Aluminium, das im Wesentlichen gleichmäßig mit den Aluminiumoxid-Teilchen verteilt ist, wobei mindestens 80% der Aluminiumoxid-Teilchen gleichmäßig auf einer Skala des Dreifachen der durchschnittlichen Teilchengröße verteilt sind, wobei die Aluminiumoxid-Keramik-Beladung 15 Vol.% bis 50 Vol.% beträgt.

## Revendications

1. Procédé de fabrication d'un composite à matrice métallique comprenant les étapes consistant à :
- fournir une préforme de céramique comportant des particules de céramique inférieures au micromètre et fritter les particules de céramique les unes aux autres ;
- disposer ladite préforme de céramique dans un moule ;
- mettre en contact ladite préforme de céramique avec un métal fondu ;
- faire pénétrer ledit métal fondu dans ladite préforme ; et
- laisser ledit métal fondu se solidifier pour former un composite à matrice métallique ;
dans lequel ledit composite à matrice métallique est usinable à l'aide d'un outil de coupe en acier rapide, **caractérisé en ce que**
lors d'une première étape, une suspension colloïdale de particules de céramique dans un liquide est soumise à une étape de broyage afin de fournir la suspension colloïdale de particules de céramique dans laquelle lesdites particules ont une taille de particule qui n'est pas supérieure au micromètre ; puis lesdites particules de céramique sont séparées du liquide pour fournir une préforme de céramique ayant une distribution uniforme desdites particules de céramique inférieures au micromètre.

2. Procédé de fabrication d'un composite à matrice métallique selon la revendication 1, dans lequel au moins 80% desdites particules de céramique sont distribuées uniformément sur une échelle de trois fois la taille. de particule moyenne.

3. Procédé de fabrication d'un composite à matrice métallique selon la revendication 2, dans lequel au moins 90% desdites particules de céramique sont distribuées uniformément sur une échelle de deux fois la taille de particule moyenne.

4. Procédé de fabrication d'un composite à matrice métallique selon la revendication 1, dans lequel l'étape consistant à laisser pénétrer ledit métal fondu dans ladite préforme est réalisée au moyen d'une infiltration sous pression.

5. Procédé selon la revendication 4, dans lequel ladite préforme de céramique comprend une porosité de 50% à 85% en volume.

6. Procédé selon la revendication 5, dans lequel ladite préforme de céramique consiste en une porosité de 60% à 80% en volume.

7. Procédé selon la revendication 4, dans lequel ledit composite possède un module de traction qui est supérieure d'au moins 30% à 200% au module de traction dudit métal.

8. Procédé selon la revendication 1, dans lequel ladite étape consistant à fournir une préforme de céramique comprend les étapes consistant à filtrer, extruder, presser ou couler en barbotine un précurseur desdites particules pour produire une préforme crue.

9. Procédé selon la revendication 1, dans lequel ladite étape de pénétration comprend une infiltration de métal fondu, lors de laquelle un gaz sous pression contraint le métal fondu à pénétrer dans les pores de ladite préforme.

10. Procédé selon la revendication 9, dans lequel ledit gaz sous pression a une pression de 6,895 MPa à 20,685 MPa (1 000 psi à 3 000 psi) et ladite préforme a une résistance à la compression d'au moins 3,448 MPa (500 psi).

11. Procédé selon la revendication 1, dans lequel ledit métal fondu est introduit dans ladite préforme au moyen d'une infiltration sous pression afin de faire pénétrer le métal fondu dans les pores de ladite préforme sans rompre ladite préforme.

12. Procédé selon la revendication 11, dans lequel les particules de céramique comprennent : un oxyde, un borure, un nitrure, un carbure, un carbone, un siliciure, un sulfure, un oxysulfure ou un mélange de ceux-ci.

13. Procédé selon la revendication 11, dans lequel la suspension colloïdale des particules de céramique est mélangée à une charge, un liant ou un mélange de ceux-ci jusqu'à un volume de 70% par rapport au volume des ingrédients secs.

14. Procédé selon la revendication 10, dans lequel ledit gaz sous pression est un gaz inerte ayant une pression de 10,34 MPa à 17,23 MPa (1 500 psi à 2 500 psi).

15. Procédé selon la revendication 11, dans lequel ledit composite à matrice métallique est proche de sa dimension finale.

16. Procédé selon la revendication 1, dans lequel ledit métal fondu est choisi dans le groupe formé par : Al, Li, Be, Pb, Ag, Au, Sn, Mg, Ti, Cu, Zn ou un mélange de ceux-ci.

17. Procédé selon la revendication 1, dans lequel ladite étape consistant à fournir une préforme comprend les étapes consistant à : filtrer sous pression un précurseur desdites particules de céramique à l'aide d'un filtre de graphite lors de l'étape de séparation, mettre en suspension lesdites particules filtrées avec une charge de graphite et un liant inorganique pour former une préforme crue ; et brûler ladite préforme crue pour éliminer ladite charge, ainsi une partie desdites particules de céramique sont frittées les unes aux autres.

18. Procédé selon la revendication 9, dans lequel ladite étape de contrainte comprend l'étape consistant à évacuer un gaz de ladite préforme en la mettant sous vide et à contraindre ledit métal fondu à pénétrer dans les pores de ladite préforme à l'aide d'un gaz contenant de l'argon sous pression.

19. Procédé selon l'une quelconque des revendications 1 à 18, dans lequel lesdites particules sont Al₂O₃ et ledit métal fondu est Al.

20. Procédé selon l'une quelconque des revendications 1 à 19, dans lequel lesdites particules ont une granulométrie allant de 0,01 micromètre à 0,5 micromètre.

21. Composite à matrice métallique comprenant une distribution uniforme de particules d'alumine ayant une taille de particule moyenne qui n'est pas supérieure au micromètre et de l'aluminium distribué essentiellement uniformément avec lesdites particules d'alumine, au moins 80% desdites particules d'alumine étant distribuées uniformément sur une échelle de trois fois la taille de particule moyenne, dans lequel la charge de céramique d'alumine va de 15% en volume à 50% en volume.
